

Patented Apr. 20, 1926.

1,581,813

# UNITED STATES PATENT OFFICE.

WALTER M. SCHMITT, OF EVANSVILLE, INDIANA.

## DECORATIVE FINISH AND PROCESS OF OBTAINING SAME.

No Drawing.

Application filed April 11, 1924. Serial No. 705,932.

To all whom it may concern:

Be it known that I, WALTER M. SCHMITT, a citizen of the United States, and a resident of Evansville, county of Vanderburg, and

5 State of Indiana, have invented a certain new and useful Decorative Finish and Process of Obtaining Same; and I do hereby declare that the following is a full, clear, and exact description thereof.

10 This invention relates to a decorative finish particularly for walnut surfaces or the like, or any other suitable material surface adapted to receive the same, and the process of securing said finish. Heretofore it has been impossible to tint walnut without partially covering or obliterating the grain.

15 The chief object of the invention is to produce "a fast to the light" or permanent decorative finish having artistic, antique and ornamental characteristics heretofore never produced or secured and which is capable of receiving any of the well known standard finishes.

20 The chief feature of the invention consists in the production of a decorative finish suitable for walnut surfaces or the like, whereby the grain of the walnut surface, either solid or veneered, is retained with all of nature's marks and beauty, and which 25 is intensified and enhanced by the addition of a variety of harmonizing shades of color substantially devoid of any opaqueness or 30 translucency and the production of a finish of the character indicated through a process 35 as hereinafter will be pointed out in detail.

40 Among the beautiful shades produced are ruby, cosine pink, apple blossom pink, lilac, orchid, Napoléon gray, olive, jade green, greenish blue and sky blue; and they as well 45 as others have been applied to solid and veneered walnut surfaces utilized for furniture of all kinds, musical instruments and interior decorations, including paneling, for public and private buildings, and for any other suitable purposes.

45 The decorative finish can be described by briefly enumerating and detailing the steps in the process.

50 After the surface has been properly prepared for finishing purposes, for example by sanding and the like, well known in the art, the dye is applied thereto. The dye consists of a suitable shade or shades of an aniline or alizarin dyestuff material, depending upon the finish or color desired 55 to be produced. This dyestuff material is

mixed with a mordant for the purpose of fixing the dye when applied to the surface. The resultant solution may be spread upon the surface with a soft brush and allowed 60 to dry, twenty-four hours standing having been found satisfactory.

The particular mordant used with the dye selected consists of a solution of a mixture of picric acid, gallic acid, sulphate of sodium 65 and chloride of sodium. Picric acid is very satisfactory in connection with chloride of sodium and sulphate of sodium. It penetrates walnut and walnut veneers more deeply than any other agent, but when used 70 alone, produces a garish appearance. Gallic acid, it has been determined, has a most kindly effect upon walnut and walnut veneers; and when mixed with the picric acid 75 has a soothing effect thereon. At the same time it takes nothing away from the "bloom" or "tone" which the picric acid imparts to the wood surface. Satisfactory results for several different shades or colors have been secured by the use of a dye material, and 80 herein, and solely for the purpose of illustration and not in any way for the purpose of limitation, a few examples of satisfactory formulas will be given.

85

### Jade green.

7/8 grain indigotine conc., 3/4 grain chloride sodium, 1/2 grain sulphate sodium, 1/2 grain gallic acid, 1/2 grain picric acid, 1 ounce water.

90

### Eosine pink.

1/8 grain orange 11, 3/8 grain carmine B. B., 1/2 grain chloride sodium, 1/4 grain sulphate of sodium, 1/4 grain gallic acid, 1/8 grain picric acid, 1 ounce water.

95

### Greenish blue.

1/8 grain erythrine pink, 1/2 grain patent blue A. D., 1 grain chloride of sodium, 1/2 grain sulphate of sodium, 1 grain gallic acid, 1/2 grain picric acid, 1 ounce water.

100

### Napoleon gray.

1 grain acid alizarine gray G., 1 grain chloride of sodium, 1/2 grain sulphate of sodium, 1 1/2 grains gallic acid, 3/4 grain picric acid, 1 ounce water.

105

### Orchid.

110

1 1/4 grains sulphon violet R., 3/4 grain sulphate of sodium, 1/2 grain chloride of

sodium,  $\frac{3}{4}$  grain gallic acid,  $\frac{3}{4}$  grain picric acid, 1 ounce water.

*Lilac.*

5  $\frac{1}{4}$  grain methylene blue Z. X.,  $\frac{1}{2}$  grain pont ruby G., 1 grain chloride of sodium,  $\frac{1}{4}$  grain sulphate of sodium,  $\frac{3}{4}$  grain gallic acid,  $\frac{1}{2}$  grain picric acid, 1 ounce water.

10 *Sky blue.*

$\frac{3}{2}$  grain carmine B. B.,  $\frac{3}{8}$  grain indigo-tine cone.,  $\frac{3}{4}$  grain chloride sodium,  $\frac{1}{2}$  grain sulphate sodium, 1 grain gallic acid,  $\frac{1}{2}$  grain picric acid, 1 ounce water.

15 *Ruby.*

1 grain ruby G., 1 grain chloride of sodium,  $\frac{1}{2}$  grain sulphate of sodium, 1 grain gallic acid,  $\frac{1}{2}$  grain picric acid, 1 ounce water.

20 These formulas may be varied within reasonable limits without departing in any way from the invention, and it will, of course, be understood that other colors may be utilized without departing from the invention, these formulas as previously stated being merely examples of what may be accomplished by the novel process, for almost any combination of shades can be produced by the use of the dyestuffs enumerated above or by other suitable dyestuffs. Darker shades can be produced by using stronger solutions, and, therefore, the percentages herein given are not to be considered in any way other than illustrative. After the dye and mordant has been spread and dried upon the surface, the same may be further prepared as by sanding and the like. A satisfactory mellowing agent has been prepared, and this includes amyl acetate, gallic acid and benzoic acid. An alcoholic solution of the foregoing mixture is used as a diluent upon a lacquer until the desired consistency is attained which permits the resultant to be readily worked. The proportions are about four to one, although they may be varied as desired. The lacquer is an American made product and a derivative of gun cotton and is commercially common in the art. When the lacquer contains impurities such as copper or iron, the same turns brown on the addition of the first-mentioned acid and acetate mixture, and, therefore, a relatively pure lacquer is preferred, and one of which is commercially marketed at the present time is of this character. Solely by way of an indication of a satisfactory mixture of acid and acetate, the following is given:

25 2 ounces amyl acetate, 4 ounces denatured alcohol, 32 grains gallic acid, 32 grains benzoic acid.

The amyl acetate utilized seems to form an excellent combining agent for the ben-

zoic acid and the lacquer, said acetate being 65 of acid tendency and of an oily nature as well.

This mellowing agent of the general character indicated mellows the shade of the dye thus fixed, tones down the garishness of it 70 and also evens it. Most acids have an undesirable effect on the dyestuffs. Picric acid usually leaves a yellowish cast but sometimes a reddish cast. It has been found that benzoic acid counteracts this undesirable casting 75 effect. Gallic acid utilized in this second step of the process further mellows the product and enhances the antique effect.

The mellowing agent previously described, by reason of the presence of the lacquer in 80 the same, in addition to performing the foregoing mellowing and toning functions also forms a protective coating which protects the underlying or color coat, secured through the first step of the process including application of the dye, from the material used in the third step or subsequent stage or stages hereinafter to be indicated. Without the lacquer or an equivalent intermediate coat the materials of the first step 85 and the application of the third step would intermingle and the latter would coat and smear them over, which would largely destroy the bloom, tone and beauty secured by the first step. If the pores of the wood 90 surface are not open, the same is suitably prepared to open said pores, although generally the wood is of such a nature that the pores are already open. The gallic acid has strong astringent properties, and its use 100 in both the first and second steps of the process, in addition to other functions, causes the closure of the pores and as quickly as possible, thereby insuring an evener surface and a closer retention of the dyestuffs utilized. Tannic acid and pyrogallic acid have been utilized and will produce similar but not as satisfactory results, for they do not produce quite as mellow and antique effects as the gallic acid produces. 105 The substitution of pyrogallic acid for gallic acid, and tannic acid for gallic acid, or a mixture of both for gallic acid, or a combination of the three acids, is to be considered as equivalent where the claim or 110 claims specifies gallic acid.

115 After the resultant is spread rapidly and evenly over the surface, the same is permitted to dry, following which the surface is again prepared as hereinbefore indicated 120 by sanding and the like, a common practice in the art. After such preparation, there is applied to said surface a filler, the application of which is intended to fill all of the fine pores that are in the surface and make a substantially smooth and even surface. A satisfactory filler material has been prepared as follows: To silicon dioxide in pow-

dered form is mixed linseed oil or any other suitable material to secure a mixture having the consistency of heavy paste. Anilines or alizarines of various shades are dissolved in a mixture of turpentine and benzine of which the following proportions are given by way of example: turpentine 2 drams, benzine, 6 drams, dyestuff as desired, 4 grains, which makes about one ounce of material that must be frequently shaken. The dye solution is added to the heavy paste until the whole is of the desired shade and the proper consistency to be handled. The dyestuff used in the formation of the filler material is an entirely different group from those used in the preparation of the first dye or step of the process. It may be possible that in some instances the same dyestuff may be utilized. However, great care must be exercised to have the filler the exact shade of the first coat; otherwise, the finished surface will show up in fine specks where the filler is fixed in the pores of the surface.

25 The filler material is then applied to the surface prepared as aforesaid and is allowed to dry as is the usual practice following which it is rubbed off in the usual way well known in the art. The surface thus treated is then permitted to stand for sometime, generally over night being sufficient.

After the filler has been applied to the surface and has been treated as indicated or in any other desired manner, said surface is provided with a suitable protective coating which may be made up of several coats of varnish, shellac, lacquer, wax or the like applied in a well known manner to obtain the usual desired final finish known to the trade. Other suitable and desirable finishes may be applied instead of the foregoing, and these may be commonly known in the art or may be special finishes that will be satisfactory.

45 Contrary to the usual results obtained with enamels and the like the decorative finish, formed by the three steps of the process hereinbefore described, permits the grain of the surface to be plainly visible through said finish. The general characteristic of the finish in addition to the substantially complete visibility of the grain therethrough is the delicate tinting of the surface and also the variegated tinting thereof, whereby the desired aesthetic, beautiful and harmonious result is attained. The colors while full in tone are light and delicate in shade and are substantially free from any undesirable by-effects of the chemicals utilized which might have a tendency

to exaggerate the same and in some instances will destroy the beauty of the final product.

While the invention has been described in great detail in the foregoing specifications, the many modifications thereof which will readily suggest themselves to those skilled in the art to which this invention applies, as well as the many modifications which have been suggested herein, all are to be considered within the broad purview of this invention, reference being had to the appended claims; and furthermore, the detailed description and specific proportions hereinbefore enumerated are to be considered, unless otherwise specifically mentioned in the particular claim, as being merely illustrative and in no way restrictive of the generic invention.

The invention claimed is:

1. The process of forming a decorative finish for wood including coating the article to be finished by dyeing and mordanting the same, and applying thereto a mellowing coat including gallic and benzoic acids.

2. In the process of forming a decorative finish for a dyed wood article, the step of mellowing the dyed portion by applying a mellowing coat including gallic acid and benzoic acid.

3. The process of forming a decorative finish for wood including coating the article to be finished by dyeing and mordanting the same to the desired tint and applying thereto a mellowing coat of substantially the same tint as the mordanted dyed coat, said mellowing coat including gallic and benzoic acids.

4. The process of forming a decorative finish for wood including coating the article to be finished by dyeing and mordanting the same to the desired tint and applying thereto a mellowing coat of substantially the same tint as the mordanted dyed coat, said mellowing coat including gallic and benzoic acids, and subsequently applying a filler of substantially the same tint as the mellowed, mordanted dyed coat.

5. An initially grained and textured walnut surfaced article having a tinted coating, said coating including the reaction products resulting from the use of picric, gallic and benzoic acids.

6. A toning solution of the character described for a dyed walnut surface including an alcoholic solution of benzoic acid, amyl-acetate, gallic acid and lacquer.

In witness whereof, I have hereunto affixed my signature.

WALTER M. SCHMITT.